

Dec. 20, 1932.

E. C. CROCKER

1,891,258

METHOD FOR FLAMEPROOFING COMBUSTIBLE MATERIALS  
AND PRODUCT RESULTING THEREFROM  
Filed Feb. 14, 1924



Tracer:

E. C. Crocker

by Huber, Huber & Cushing  
Rec'd Oct 5.

## UNITED STATES PATENT OFFICE

ERNEST C. CROCKER, OF BELMONT, MASSACHUSETTS, ASSIGNOR TO ARTHUR D. LITTLE, INCORPORATED, OF CAMBRIDGE, MASSACHUSETTS, A CORPORATION OF MASSACHUSETTS

**METHOD FOR FLAME-PROOFING COMBUSTIBLE MATERIALS AND PRODUCT RESULTING THEREFROM**

Application filed February 14, 1924. Serial No. 692,914.

This invention relates to substances, including electrical insulators, so modified or treated as to inhibit the propagation of flame, and to a way of treating such substances adapted to reach these results.

With many commercial materials which are inherently combustible (but which are, on account of other valuable properties, preferable to non-combustible substances for their several uses) it is desirable and sometimes required by regulatory statutes that the materials shall be flame proof. By "flame proof" is meant a quality causing ignition of the material to be more difficult and the natural tendency of the material to support progressive combustion to be measurably diminished or more or less completely suppressed. Treatment to cause the materials to have these qualities is known as flame proofing.

In such cases, it is not always desirable to so completely alter the characteristics of the material as to render it absolutely fireproof or non-combustible though in special instances this degree of protection may be advantageously effected.

Heretofore, the expedients resorted to for this purpose have generally consisted in impregnating the material with a non-combustible salt or compound which, upon becoming heated, is intended either to dissociate into a non-combustible gas or flux over the surface, sealing the interior of the material from contact with the air. A common objection to such treatment is that the supposed functions of the compounds used are only partially effective in practice and secondly, that such compounds are electrical conductors and not sufficiently inert chemically.

Combustion being a rapid oxidation of a substance which takes place at or above a given temperature dependent upon the character of the substance, progressive combustion or flame propagation requires that this temperature be maintained and transferred, and that a continued interaction between oxygen (as of air) and the substance in question, shall take place.

The materials thus far used for flame proofing have not affected the first men-

tioned requisite for propagating combustion and have counteracted the second only to a slight degree as by flowing over the heated area and excluding the air or by diluting the air with a non-combustible gas such as ammonia.

This invention proceeds upon the discovery that certain materials when raised to the temperature of combustion in air will ignite, and therefore deplete the oxygen of the air in contact, but nevertheless will fail to rise in temperature as a result of combustion sufficiently to maintain, or to propagate in themselves, a temperature sufficiently elevated to continue their own combustion. When exposed to conditions of elevated temperature, such materials may be expected to inhibit flame, of themselves or their environing combustibles. If the oxide of the material chosen should form a vapor at a relatively low temperature, the result is further to inhibit flame by the formation of a zone of non-combustible vapor.

I have discovered that the element selenium, for example, although itself combustible, has the property of inhibiting, even when present in relatively minute quantity, the combustion of otherwise combustible material with which it is associated, as for example fabrics or structures of vegetable fibers. Furthermore, the element imparts this property to certain at least of its compounds, this being true of sodium selenite, selenious and selenic acids among others, so that materials so protected by the element or its compounds are thereby rendered flame proof.

The present invention accordingly comprises the treatment of a combustible material with a suitable compound or material of the class indicated for the purpose of rendering such material difficult of ignition or flame proof. The treatment may be effected in any suitable manner, but it is preferable to use the substance in finely divided condition and to impregnate or coat the surface therewith either in powder form or in the form of a liquid suspension, solution or paint.

A typical example of the application of the invention will be described in relation to

flame proofing electrically insulated wire with a powdered substance adapted to produce the required effects, for which purpose the element selenium is peculiarly effective.

5 Such wire ordinarily has a covering of rubber and an outer covering of a textile such as paper or cotton, braided, wound or otherwise applied. The treatment may be carried out upon the wire either before or after the textile covering has been applied or it may be applied to the covering itself.

10 For the purpose of explaining the invention, the accompanying drawing in the nature of a diagram illustrates one flame-proofed article, an insulated wire, by way of specific exemplification of the genus of such articles within the invention. In this drawing, the figure is an elevation partly in section.

15 The particular manner of applying the flame proofing material may be varied according to the specific conditions to be encountered. In some instances it may be found practicable to merely cover the wire with the finely divided element alone, as by 20 dusting or compressing a powder of the element into the surface of the material, and then making the textile cover around it.

25 A procedure which is generally preferable, consists in preparing a paste, for example, 30 with a water solution of dextrine and powdered selenium, preferably the amorphous gray allotropic form (150-300 mesh), substantially in the following proportions by weight:

35                   7 parts water  
                      5 parts dextrine  
                      5 parts selenium

40 The wire 1, already covered by the plastic or gummy flexible insulating coat 2, such as one of the rubber compounds, is then drawn through the mixture, a thin layer 3 of which will adhere to the surface. A textile cover 4 for example of cotton, paper ramie, or silk may then be braided or otherwise applied 45 over the exterior surface, and the treating mixture will serve to retain the covering thereon as well as to hold the selenium powder in suspension. Upon drying, the selenium will remain in a uniformly distributed layer 50 between the fabric covering 4 and the gummy insulation 2.

55 If a wire so treated is ignited the textile elements of the cover will burn in the area so ignited. However, the flame will not spread beyond this area, but presently the incandescent portion is found to be separated from the wire, leaving a zone of substantial extent (which is relatively cool) between the incandescent portion and the wire, which zone 60 gradually widens, and the flame, thus removed from the wire, goes out.

65 Whatever the nature of the combustion tests on the described specific instance of the article of manufacture of this invention, there is visible evidence of the formation of red

vapors presumably containing selenium oxide or selenium or both, and possibly selenium nitride, these vapors constituting a combustion-inhibiting zone of appreciable extent which rapidly develops after the initial ignition of the combustible elements of the wire. 70

Another feature of the invention is demonstrated by comparison of a treated wire according to this invention with the behavior of insulated wires otherwise treated. 75 The latter when ignited and extinguished at one point are found to have lost their "flame proof" characteristic in lengths adjacent to the portion so tested. When treated in accordance with the present invention the testing of one portion in this manner does not diminish in any wise the effective protection of any other part of the wire. 80

85 It will now be clear that whatever the true explanation of the observed phenomena, the mode of treatment and the resulting article of this invention is useful wherever flame-proofed combustibles may desirably be employed. While a preferred material and an important use have been described, the invention is generally applicable to the flame-proofing of combustible materials. 90

95 Compounds of selenium, in the practice of the invention, may be employed either in solution or in comminuted form with much the same effect. For example, selenium oxychloride, sodium selenite, selenious acid and selenic acid, although not quite so advantageous as the elemental substance, may be employed with beneficial effect. It will be 100 observed that these substances are adapted to reduce to elemental selenium on the application of heat, whereupon the resultant behavior of the selenium accrues, with the effect of the elemental application. 105

110 I am not to be understood as excluding other elements than selenium or the alloys or simple compounds of elements, since it is obvious that any substance, capable of combining directly with oxygen (of the air) but not of supporting its own combustion (and having as well the other properties made use of in the instance of selenium, such as non-volatility at ordinary temperature but appreciable volatility at the combustion temperature of the material flame proofed) will be effective if not disqualified for other reasons. Arsenic is an example of such an element. The extremely poisonous character of its compounds, however, precludes its use in 115 many usual situations.

I claim:

1. An insulated wire having a portion including selenium for flame proofing.
2. An insulated wire flame proofed with a substance containing selenium carried co-extensively with the extent of the wire. 125
3. A flame-proofed material having distributed thereon finely divided selenium.
4. A flame-proofed material having dis- 130

tributed thereon selenium in its gray allotropic form.

5. A flame-proofed material having distributed thereon a substance containing ele-  
5 mentary selenium at the temperature of com-  
bustion of the material.

6. A flame-proofed material having dis-  
tributed thereon a finely divided substance  
containing selenium.

10 7. A combustible material flame-proofed  
by a coating containing selenium.

8. A combustible material flame-proofed  
by a coating containing selenium and an-  
other substance.

15 9. A combustible material flame-proofed  
by a coating containing selenium and oxygen.

10. Combustible material flame-proofed by  
the presence thereon of a suspension of finely  
communited gray selenium in an organic sub-  
20 stance.

25 11. An insulated wire comprising a core  
of electrically conducting material, a coating  
of insulating material applied thereover, a  
second coating comprising selenium and a  
binding medium applied over said first-men-  
tioned coating, and a textile covering applied  
over said second coating.

30 12. An insulated wire comprising a core  
of electrically conducting material having a  
coating of rubber insulating material applied  
thereon, and a second coating including se-  
lenium applied directly on said first-men-  
tioned coating to render the insulated wire  
resistant to flame.

35 13. A flame-proof insulated wire having a  
coating comprising selenium and a binding  
medium applied on rubber insulation.

Signed by me at Cambridge, Massachu-  
sets, this 12th day of February, 1924.

40 ERNEST C. CROCKER.